

## UNITED STATES PATENT OFFICE

2,246,134

## HEAT TREATMENT FOR ALUMINUM BASE ALLOYS

Richards H. Harrington, Schenectady, N. Y., assignor to General Electric Company, a corporation of New York

No Drawing. Application July 29, 1938,  
Serial No. 221,975

2 Claims. (Cl. 148—21.1)

The present invention relates to heat treatment for aluminum base alloys and more particularly to a heat treatment for aluminum alloys containing more than 90% aluminum with the remainder either silicon and magnesium, or silicon, magnesium and copper. Heretofore the heat treatment applied to alloys consisting of aluminum, silicon and magnesium comprised heating the castings for approximately twelve hours at 538° C. to effect a solution condition in the alloy, quenching, and reheating for about three to five hours at 160° C. to effect a condition of precipitation. The properties resulting from the application of such a heat treatment to castings consisting of 7% silicon, 0.3% magnesium and the remainder aluminum are substantially as follows:

## Proportional limit

|                  |          |        |
|------------------|----------|--------|
| Yield strength   | do       | 22,000 |
| Tensile strength | do       | 31,000 |
| Elongation       | per cent | 3 to 4 |

It is one of the objects of the present invention to provide a heat treatment for aluminum base alloys whereby the physical properties of such alloys may be improved.

In carrying out the present invention, I have found that the above properties of such alloys may be greatly improved if the castings are heated at 530° C. for two to four hours, quenched, and then reheated for ten to twenty hours at 155° C.

Castings similar to the above-noted castings, when given my improved heat treatment, have the following properties:

## Proportional limit

|                  |          |                  |
|------------------|----------|------------------|
| Yield strength   | do       | 28,000           |
| Tensile strength | do       | 37,000 to 40,000 |
| Elongation       | per cent | 3 to 4           |

Numerous tests have indicated that the solution temperature and the time the alloy is held at that temperature are critical. Any deviation from the solution temperature greater than plus or minus 5° C. results for example in greatly lowered tensile properties in the alloy. Furthermore, any prolonged time at the solution temperature is detrimental to elongation and shock resistance. Two hours at the solution temperature is satisfactory except for very large castings which might be heated four hours. Heating for a longer period does not improve properties and leads to grain growth which is harmful. Also, the time should be as short as possible to reduce warping. The precipitation reheat temperature of 155° C. and the time at that temperature are also somewhat critical but small deviations in reheat temperature are not harmful to the same

degree as in the solution temperature. For example variations of  $\pm 10^\circ$  C. in the reheat temperature do not result in a serious loss of properties in the alloy. A reheat period of less than ten hours tends to lower the elongation to about 2% while a period greater than twenty hours effects no practical improvement.

While I prefer to employ an alloy having the above noted composition, my method is not restricted to that specific composition but may be applied to aluminum base alloys containing silicon, magnesium and copper. Alloys of this latter composition heretofore have been heat treated to improve their physical properties, the heat treatment comprising heating for twenty hours at 520° C., quenching in water and reheating four hours at 155° C. Such a heat treatment does not develop the maximum physical properties in the alloy. I have found that when alloys of the above composition are given my improved heat treatment, for example heating at 530° C. for about two hours, quenching, and then reheating from ten to twenty hours at 155° C., the physical properties of the alloys are greatly improved.

Alloys consisting of 5% silicon, 0.5% magnesium, 1.3% copper and 93.2% aluminum, when heat treated in accordance with the prior process, have the following properties:

## Proportional limit

|                  |          |        |
|------------------|----------|--------|
| Tensile strength | do       | 38,200 |
| Elongation       | per cent | 6      |

The same alloys, when heat treated in accordance with my improved process, have the following properties:

## Proportional limit

|                  |          |         |
|------------------|----------|---------|
| Tensile strength | do       | 43,100  |
| Elongation       | per cent | 3.5—4.5 |

What I claim as new and desire to secure by Letters Patent of the United States, is:

1. The method of heat treating aluminum base alloys containing about 7% silicon, about 0.3% magnesium and the remainder substantially aluminum which comprises heating the alloy at a temperature of 530° C. for about two hours, quenching and reheating at 155° C. for at least ten hours.

2. The method of heat treating aluminum base alloys containing about 5% silicon, about 0.5% magnesium, about 1.3% copper and the remainder substantially aluminum, which comprises heating the alloy at a temperature of 530° C. for about two hours, quenching and reheating at 155° C. for at least ten hours.

RICHARDS H. HARRINGTON.